



linkages. This may be further demonstrated by a few specific examples which fall into these classes, thus

*Class A esters*, e.g.:



5

10

which are derivatives of alcohols of the formula  $\text{R}_d\text{CH}_2\text{OH}$ .

*Class B esters*, e.g.:



15

20

which are derivatives of acids of the formula  $\text{R}_d\text{COOH}$ .



4

which are derivatives of either the alcohols of the formula  $\text{R}_d\text{CH}_2\text{OH}$  or their halides,  $\text{R}_d\text{CH}_2\text{X}$ .

*Class D hydrocarbons*, e.g.:



which are derivatives of either the alcohol  $\text{R}_d\text{CH}_2\text{OH}$  through standard alkylation or derivatives of the halide  $\text{R}_d\text{CH}_2\text{X}$  through standard alkylation or Grignard reaction. In the event the hydrocarbon group is attached to the aromatic nucleus by alkylation the group is generally attached through the second carbon atom from the end of the aliphatic chain.

Preferred Z groups are defined in the following tables which illustrate structures of the monomers of this invention:

|                                    | Z                                                                          |                              |
|------------------------------------|----------------------------------------------------------------------------|------------------------------|
| $\text{CH}_2=\text{CR}-\text{Ar}-$ | $-\text{COO}-$                                                             | $-\text{CH}_2\text{R}_d$     |
| $\text{CH}_2=\text{CR}-\text{Ar}-$ | $-\text{COO}(\text{CH}_2)_n\text{O}-$                                      | $-\text{CH}_2\text{R}_d$     |
| $\text{CH}_2=\text{CR}-\text{Ar}-$ | $-\text{COO}(\text{CHRCHRO})_n-$                                           | $-\text{CH}_2\text{R}_d$     |
| $\text{CH}_2=\text{CR}-\text{Ar}-$ | $-(\text{CH}_2)_n\text{COO}-$                                              | $-\text{CH}_2\text{R}_d$     |
| $\text{CH}_2=\text{CR}-\text{Ar}-$ | $-(\text{CH}_2)_n\text{COO}(\text{CH}_2)_n\text{O}-$                       | $-\text{CH}_2\text{R}_d$     |
| $\text{CH}_2=\text{CR}-\text{Ar}-$ | $-(\text{CH}_2)_n\text{COO}(\text{CHRCHRO})_n-$                            | $-\text{CH}_2\text{R}_d$     |
| $\text{CH}_2=\text{CR}-\text{Ar}-$ | $-\text{O}-$                                                               | $-\text{CH}_2\text{R}_d$     |
| $\text{CH}_2=\text{CR}-\text{Ar}-$ | $-\text{O}(\text{CH}_2)_n\text{O}-$                                        | $-\text{CH}_2\text{R}_d$     |
| $\text{CH}_2=\text{CR}-\text{Ar}-$ | $-\text{O}(\text{CHRCHRO})_n-$                                             | $-\text{CH}_2\text{R}_d$     |
| $\text{CH}_2=\text{CR}-\text{Ar}-$ | $-(\text{CH}_2)_n\text{O}-$                                                | $-\text{CH}_2\text{R}_d$     |
| $\text{CH}_2=\text{CR}-\text{Ar}-$ | $-(\text{CH}_2)_n\text{O}(\text{CH}_2)_n\text{O}-$                         | $-\text{CH}_2\text{R}_d$     |
| $\text{CH}_2=\text{CR}-\text{Ar}-$ | $-(\text{CH}_2)_n\text{O}(\text{CHRCHRO})_n-$                              | $-\text{CH}_2\text{R}_d$     |
| $\text{CH}_2=\text{CR}-\text{Ar}-$ | $-\text{NR}(\text{CH}_2)_n\text{COO}-$                                     | $-\text{CH}_2\text{R}_d$     |
| $\text{CH}_2=\text{CR}-\text{Ar}-$ | $-\text{NR}(\text{CH}_2)_n\text{COO}(\text{CH}_2)_n\text{O}-$              | $-\text{CH}_2\text{R}_d$     |
| $\text{CH}_2=\text{CR}-\text{Ar}-$ | $-\text{N}(\text{CHR}(\text{COO}))_2-$                                     | $(-\text{CH}_2\text{R}_d)_2$ |
| $\text{CH}_2=\text{CR}-\text{Ar}-$ | $-\text{OCH}_2\text{CH}-\text{O}-$                                         | $-\text{CH}_2\text{R}_d$     |
|                                    | $\quad \quad \quad \text{CH}_2\text{OC(O)R}'$                              |                              |
| $\text{CH}_2=\text{CR}-\text{Ar}-$ | $-\text{OCH}_2\text{CHCH}_2\text{O}-$                                      | $-\text{CH}_2\text{R}_d$     |
|                                    | $\quad \quad \quad \text{O C(O)R}'$                                        |                              |
| $\text{CH}_2=\text{CR}-\text{Ar}-$ | $-\text{CH}-\text{CH}_2\text{O}-$                                          | $-\text{CH}_2\text{R}_d$     |
|                                    | $\quad \quad \quad \text{O C(O)R}'$                                        |                              |
| $\text{CH}_2=\text{CR}-\text{Ar}-$ | $-\text{CH}-\text{O}-$                                                     | $-\text{CH}_2\text{R}_d$     |
|                                    | $\quad \quad \quad \text{CH}_2\text{OC(O)R}'$                              |                              |
| $\text{CH}_2=\text{CR}-\text{Ar}-$ | $-(\text{CH}_2)_n\text{O}\text{C(O)}-$                                     | $-\text{R}_d$                |
| $\text{CH}_2=\text{CR}-\text{Ar}-$ | $-(\text{CH}_2)_n\text{O}(\text{CH}_2)_n\text{O}\text{C(O)}-$              | $-\text{R}_d$                |
| $\text{CH}_2=\text{CR}-\text{Ar}-$ | $-(\text{CH}_2)_n\text{O}(\text{CHRCHRO})_n\text{C(O)}-$                   | $-\text{R}_d$                |
| $\text{CH}_2=\text{CR}-\text{Ar}-$ | $-(\text{O}(\text{CH}_2)_n\text{O})-$                                      | $-\text{R}_d$                |
| $\text{CH}_2=\text{CR}-\text{Ar}-$ | $-(\text{O}(\text{CH}_2)_n\text{O}(\text{CHRCHRO})\text{C(O)})-$           | $-\text{R}_d$                |
| $\text{CH}_2=\text{CR}-\text{Ar}-$ | $-(\text{O}(\text{CHRCHRO})\text{C(O)})-$                                  | $-\text{R}_d$                |
| $\text{CH}_2=\text{CR}-\text{Ar}-$ | $-(\text{NR}(\text{CH}_2)_n\text{COO}(\text{CH}_2)_n\text{O}\text{C(O)})-$ | $-\text{R}_d$                |
| $\text{CH}_2=\text{CR}-\text{Ar}-$ | $-(\text{NR}(\text{CH}_2)_n\text{COO}(\text{CHRCHRO})_n\text{C(O)})-$      | $-\text{R}_d$                |
| $\text{CH}_2=\text{CR}-\text{Ar}-$ | $-(\text{CH}_2)_n-$                                                        | $-\text{R}_d$                |
| $\text{CH}_2=\text{CR}-\text{Ar}-$ | $-\text{OCH}_2\text{CH}-\text{CH}_2\text{OC(O)}-$                          | $-\text{R}_d$                |
|                                    | $\quad \quad \quad \text{O C(O)R}'$                                        |                              |
| $\text{CH}_2=\text{CR}-\text{Ar}-$ | $-\text{OCH}_2\text{CH}-\text{O C(O)}-$                                    | $-\text{R}_d$                |
|                                    | $\quad \quad \quad \text{CH}_2\text{OC(O)R}'$                              |                              |
| $\text{CH}_2=\text{CR}-\text{Ar}-$ | $-\text{CHCH}_2\text{OC(O)}-$                                              | $-\text{R}_d$                |
|                                    | $\quad \quad \quad \text{O C(O)R}'$                                        |                              |
| $\text{CH}_2=\text{CR}-\text{Ar}-$ | $-\text{CH}-\text{O C(O)}-$                                                | $-\text{R}_d$                |
|                                    | $\quad \quad \quad \text{CH}_2\text{OC(O)R}'$                              |                              |
| $\text{CH}_2=\text{CR}-\text{Ar}-$ | $-\text{CH}(\text{CH}_3)-$                                                 | $-\text{R}_d$                |
| $\text{CH}_2=\text{CR}-\text{Ar}-$ | $-\text{CH}_2-$                                                            | $-\text{R}_d$                |

*Class C esters*, e.g.:



While the above preferred compounds have  $-(\text{CH}_2)_n$  and  $-\text{CH}_2\text{R}_d$  groups in which R is hydrogen or methyl, it is also possible to use similar alkylene groups which have a lower alkyl side branch, that is, up to 4 carbon atoms. Moreover, while glyceryl derivatives are shown and are preferred, equivalent groups such as derived from penta-erythritol and other polyhydric alcohols can also be used.

Specific typical compounds illustrative of the monomers of this invention are those of the above formulas in which  $Ar$  is the phenylene-group,  $-\text{CH}_2\text{R}_d$  is the linoleyl alcohol radical and  $Z$  is:



Other typical monomeric compounds are those in which tolylene, naphthylene, xylylene, diphenylene and chlorophenylene radicals are substituted in the above compounds for the phenylene group. Likewise other typical monomers are those in which the linoleyl alcohol radical is replaced by oleyl, linoleyl, licanyl, eleostearyl, palmitoleyl alcohol radicals, etc.

Other specific typical monomers are those of the above formulas in which  $Ar$  is phenylene,  $R_d$  is the hydrocarbon portion of linoleic acid and the  $Z$  radical is as follows:



The monomers of this invention are readily prepared through classical organic reactions when based on alcohols, acids, and halides of the formulas  $R_dCH_2OH$ ,  $R_dCOOH$ , and  $R_dCH_2X$  respectively, as illustrated by the following examples. The Class A esters are readily prepared by reacting an  $R_dCH_2OH$  alcohol with an appropriate vinyl aryl carboxy compound as illustrated by vinyl benzoic acid compounds e.g.



wherein R' is hydrogen or a hydrocarbon radical containing one to twelve carbon atoms. In this reaction the preferred groups for R' are hydrogen and the lower alkyl radicals containing one to four carbon atoms, e.g., H,  $\text{CH}_3$ ,  $\text{C}_2\text{H}_5$ ,  $\text{C}_3\text{H}_7$ , and  $\text{C}_4\text{H}_9$ .

Another convenient method of preparing these esters is to react the acid chlorides with the alcohols in the presence of a hydrohalide acceptor (HAC) such as triethyl amine, tributyl amine, pyridine,  $\text{Na}_2\text{CO}_3$ , etc., according to the reaction, e.g.,



Alternately, the acid anhydrides may be used, thus,  

$$(\text{CH}_2=\text{CHC}_6\text{H}_4\text{CO})_2\text{O} + \text{R}_d\text{CH}_2\text{OH} \rightarrow$$

While the vinyl benzoyl derivative is used to illustrate the ester formation, it is used only to typify the other acids falling within the scope of this invention, and the acid-alkyl esters and acid chlorides of the other acids

are also used, for example,  $\text{CH}_2=\text{CHC}_6\text{H}_4\text{CH}_2\text{COOH}$  (from  $\text{CH}_2=\text{CHC}_6\text{H}_4\text{CH}_2\text{Cl}$  with  $\text{NaCN}$  and  $\text{H}_2\text{O}$ );  $\text{CH}_2=\text{CHC}_6\text{H}_4\text{OCH}_2\text{COOH}$  (from  $\text{CH}_2=\text{CHC}_6\text{H}_4\text{ONa}$  and  $\text{CICH}_2\text{COOH}$ );  $\text{CH}_2=\text{CHC}_6\text{H}_4\text{NHCH}_2\text{COOH}$  (from  $\text{CH}_2=\text{CHC}_6\text{H}_4\text{CH}_2\text{Cl} + \text{HN}(\text{CH}_3\text{COONa})$ , etc. Typical examples of  $\text{R}_6\text{CH}_2\text{OH}$  alcohols used in the esterification are

- 10 (a) 9,12 linoleyl alcohol,  
 $\text{CH}_3(\text{CH}_2)_3(\text{CH}_2\text{CH}=\text{CH})_2(\text{CH}_2)_7\text{CH}_2\text{OH}$

(b) Linolenyl alcohol,  
 $\text{CH}_3(\text{CH}_2\text{CH}=\text{CH})_3(\text{CH}_2)_7\text{CH}_2\text{OH}$ ,

(c) Arachidonyl alcohol,  
 $\text{CH}_3(\text{CH}_2)_3(\text{CH}_2\text{CH}=\text{CH})_4(\text{CH}_2)_3\text{CH}_2\text{OH}$ ,

15 (d) Licanyl alcohol,  $\text{CH}_3(\text{CH}_2)_3(\text{CH}=\text{CH})_2(\text{CH}_2)_4\text{CO}(\text{CH}_2)_2\text{CH}_2\text{OH}$ ,

(e) Parinaryl alcohol,  
 $\text{CH}_3\text{CH}_2(\text{CH}=\text{CH})_4(\text{CH}_2)_7\text{CH}_2\text{OH}$ ,

(f) Eleostearyl alcohol,  
 $\text{CH}_3(\text{CH}_2)_3(\text{CH}=\text{CH})_3(\text{CH}_2)_7\text{CH}_2\text{OH}$ ,

20 (g) 9,11 linoleyl alcohol,  
 $\text{CH}_3(\text{CH}_2)_5(\text{CH}=\text{CH})_2(\text{CH}_2)_7\text{CH}_2\text{OH}$ .

These alcohols are obtained by catalytic reduction with hydrogen, or by chemical reduction methods as by the Beauvau Blanc reaction of an alcohol such as butyl alcohol with sodium, or by lithium hydride, etc., of the corresponding fatty acids, or their natural or synthetic esters, all of which can be represented by the reduction of methyl or glyceryl linoleate, whereby the linoleic acid moiety is reduced to the corresponding alcohol, thus



and



It will be observed that the seven alcohols (a) to (g) listed above contain at least two  $-\text{CH}=\text{CH}-$  unsaturated structures; in the first three, (a) to (c), the double bonds are not conjugated whereas in (d) to (g), the double bonds are conjugated. By subjecting esters of the type used in this invention to a directed polymerization, fully described hereinafter, they are polymerized to linear form.



with the Ar-Z group pendant to the polymer backbone. In this class of polymers, it is observed that when the  $R_d$  group contains conjugated unsaturation, more rapid air-drying is achieved than when the double bonds are not conjugated.

For very rapid drying, those polymers in which at least some of the  $R_d$  groups contain conjugated unsaturation are preferred. When very fast or very rapid drying rates are not required in the coating composition, practical and satisfactory compositions can be prepared from the monomers in which  $R_d$  contain only one  $-\text{CH}=\text{CH}-$  group. Illustrative of such alcohols containing only one  $-\text{CH}=\text{CH}-$  group from which the esters are prepared are



all of which are obtainable by reduction of the corresponding acids or esters.

It is readily observable that in these monoolefinic and polyolefinic alcohols that (1) there is no terminal  $\text{CH}_2=\text{C}$  structure, rather the terminal group is a  $\text{CH}_3-$  group, (2) the first double bond in the structure is removed from the oxygen atom of the alcohol (and therefore in its esters) by at least 4 carbon atoms and by as many as 14 carbon atoms, and therefore are not activated by the ester structure, (3) the first double bonds are removed by at least 1 carbon atom from the terminal  $-\text{CH}_3$  group which is not an activating group, and (4) there may be 1 to 4  $-\text{CH}=\text{CH}-$  groups in the unsaturated portion of the alcohol molecule. In these respects the polymers of the aryl esters of these alcohols are similar in character to the structures of drying oil and are in contrast to polymers of the allyl and methyl acrylic esters which do not air dry. The radical  $R_d$  of the  $R_d\text{CH}_2\text{OH}$  alcohols used in the preparation of these esters may be described as an unsaturated fatty or aliphatic hydrocarbon containing 15 to 23 carbon atoms, a terminal  $-\text{CH}_3$  group, 1 to 4  $-\text{CH}=\text{CH}-$  groups and the remainder being  $-\text{CH}_2-$  groups. In some cases, one  $-\text{CH}_2-$  group may be replaced, as in the case of licanic alcohol, by a keto,



group. These alcohols and their simple non-monomeric esters, such as the benzoates or tertiary butyl benzoates, do not air-dry, whereas the polymers of this invention, air-dry readily.

For the purposes of this invention the esters of pure individual alcohols are not required, although some of them have become available commercially in different degrees of purity. Mixtures of the alcohols, such as are obtained by the reduction of vegetable, animal and marine oils and fats are satisfactory. Since such oils and fats are mixtures of various glycerides, the alcohols resulting from the reduction of ester groups correspond equivalently to the amounts of acid moiety present in the glyceride. Table 1 gives the percentage composition of the fatty acids in a number of drying oils, which on reduction produce an equivalent amount of the corresponding alcohols.

TABLE 1

| Oil      | Percent of Total Fatty Acid |         |       |           |                |         |                  |
|----------|-----------------------------|---------|-------|-----------|----------------|---------|------------------|
|          | Palmitic                    | Stearic | Oleic | Lino-leic | Lino-<br>lenic | Licanic | Eleo-<br>stearic |
| Soybean  | 6.5                         | 4.2     | 33.6  | 52.6      | 2.3            | 74.1    | -----            |
| Oiticica | 5.0                         | 5.0     | 5.9   | 10.0      | -----          | 79.5    | -----            |
| Tung     | 4.0                         | 1.5     | 15.0  | -----     | -----          | 78.5    | -----            |
| Linseed  | 5.0                         | 3.5     | 5.0   | 61.5      | 25.0           | -----   | -----            |
| Perilla  | 7.5                         | -----   | 8.0   | 38.0      | 46.5           | -----   | -----            |

It will be noted in Table 1 that all of the oils have measurable amounts of compounds having one or more than one double bond in the fatty acid and therefore, the derived alcohols, since only the ester group is reduced, have a substantial amount of suitable mono- and poly-unsaturation suitable for the purposes of this invention. The alcohols derived from palmitic and stearic acids are saturated alcohols, and if present in the mixture during esterification also become converted to esters similar in structure to those of the



type and copolymerize with the



monomers, lending flexibility and ductility to the polymerization product. Mixture of such alcohols are useful

and the monomers resulting from such mixtures are also contemplated in the practice of the invention.

Instead of the alcohols  $R_d\text{CH}_2\text{OH}$ , certain derivatives of the alcohols, such as the alkylene oxide addition products can be used, and they are readily prepared by reacting the oxide with the alcohols in the presence of alkali, thus



wherein  $n$  is one to five, and if desired, may be increased, for certain application, to as high as 9 or 10. Propylene oxide and butene-2 oxide produce the corresponding alcohols,



Another class of alcoholic derivatives which can be used with the vinyl aryl carboxy compounds have the general formula,  $R_d\text{COO}-Y-\text{OH}$  as illustrated by the reaction with vinyl benzoyl chloride,



Typical examples of the  $R_d\text{COO}-Y-\text{OH}$  alcohols are  $\beta$ -hydroxyethyl linoleate,  $\beta$ -hydroxyethyl oleate and  $\beta$ -hydroxyethyl linolenate which can be represented by  $R_d\text{COOCH}_2\text{CH}_2\text{OH}$ . These hydroxy alkyl ester intermediates are prepared by esterification of the  $R_d\text{COOH}$  acids with glycols, e.g., ethylene glycol, thus



or by the reaction of the acid with ethylene oxide in the presence of a base, thus



When an excess of oxide is used for example,  $x'$  moles, when  $x'$  equals 1 to 5, then the polyoxyalkylene alcohol is obtained, e.g.,



With propylene oxide, the corresponding ester is obtained,



while styrene oxide produces a phenyl substituted derivative, thus



With trimethylene oxide or trimethylene glycol, the hydroxypropyl esters are obtained, as



Thus, it may be seen that when  $-Y-$  represents a radical of a dihydric alcohol, the intermediate



is readily prepared by esterification of only one of the hydroxy groups of the diol with an  $R_d\text{COOH}$  acid, and if the cyclic oxide corresponding to the diol is known or available, it may be used instead of the diols. The radical  $-Y-$  may also represent the radical derived from alcohols higher than the diols, such as the triols, tetrols, pentols, etc., in which case more lightly substituted derivatives falling within the general formula of the intermediates,  $R_d\text{COO}-Y-\text{OH}$  compounds are obtained.

Illustrative examples of some of the many triol, tetrol, etc. derivatives are glycerol dioleate, glycerol dilinoleate, glycerol dilinolenate, pentaerythritol trioleate, etc. The

glyceryl derivatives are readily prepared, as is known in the alkyd resin and coating arts, by transesterification of oils with glycerine, thus



which, as indicated hereinabove, are easily converted to the desired ester as is illustrated by the reaction of vinyl benzoyl chloride and glyceryl dioleate:



When —Y— is derived from a trihydric, tetrahydric, or higher alcohol, all but one of the alcoholic hydroxy groups may be esterified by the R<sub>d</sub>COOH acid and the residual hydroxyl group converted to an ester as shown with the glyceryl dioleate hereinabove and illustrated also by pentaerythritol, thus,



However, in the practice of this invention, the monomer contains only one



group and at least one R<sub>d</sub>COO— group, as illustrated with the glycols, glycerine and pentaerythritol. However, when only one of the hydroxyls in polyhydric alcohols containing more than the two —OH groups is converted to an R<sub>d</sub>COO— ester, the remaining —OH groups can be converted to groups other than R<sub>d</sub>COO groups, such as ordinary ester groups, R'COO— or ether groups, R''O—, wherein R'' is a hydrocarbon containing 1 to 18 carbon atoms, as for example,



Accordingly, these esters can also be defined as esters of polyhydric alcohols possessing two to five hydroxyl groups, said esters containing only one



group, and at least one R<sub>d</sub>COO— group. Typical exam-

ples of unsaturated R<sub>d</sub>COOH acids useful in the preparation of these hydroxylalkyl esters intermediates,



5 and from which the R<sub>d</sub>COO— group is derived, are

(a) 9, 12 linoleic acid,



(b) Linolenic acid,



(c) Arachidonic acid,



(d) Licanic acid,



(e) Parinaric acid,



(f) Eleostearic acid,



(g) 9, 11 linoleic acid,



These acids are obtained by catalytic hydrolysis with water of the corresponding natural or synthetic fatty esters, all of which can be represented by the hydrolysis of 30 methyl or glyceryl linoleate, thus



35 and



40

It will be observed that the seven acids (a) to (g) listed above contain at least two —CH=CH— unsaturated structures; in the first three (a) to (c), the double bonds are not conjugated whereas in (d) to (g), the double bonds are conjugated. As observed in the polymers derived from R<sub>d</sub>CH<sub>2</sub>OH alcohol polymers having the formula



55 and which contain an R<sub>d</sub>COO— linkage on the Z group, more rapid drying is achieved when the unsaturation in the R<sub>d</sub> group is conjugated than when it is non-conjugated. Accordingly, for very rapid drying, those polymers in which at least some of the R<sub>d</sub>COO— groups contain conjugated unsaturation are preferred,

60 When very fast or very rapid drying rates are not required in the coating composition, practical and satisfactory compositions can be prepared from the monomers in which R<sub>d</sub>COO contain only one —CH=CH— group. Illustrative of such fatty acids containing only one 65 —CH=CH— group from which the esters are prepared are

- Palmitoleic acid, (CH<sub>3</sub>)(CH<sub>2</sub>)<sub>5</sub>CH=CH(CH<sub>2</sub>)<sub>7</sub>COOH,  
 Oleic acid, CH<sub>3</sub>(CH<sub>2</sub>)<sub>7</sub>CH=CH(CH<sub>2</sub>)<sub>7</sub>COOH,  
 70 Petroselinic acid, CH<sub>3</sub>(CH<sub>2</sub>)<sub>10</sub>CH=CH(CH<sub>2</sub>)<sub>4</sub>COOH,  
 Vaccenic acid, CH<sub>3</sub>(CH<sub>2</sub>)<sub>5</sub>CH=CH(CH<sub>2</sub>)<sub>9</sub>COOH,  
 Gadoleic acid, CH<sub>3</sub>(CH<sub>2</sub>)<sub>9</sub>CH=CH(CH<sub>2</sub>)<sub>7</sub>COOH,  
 Cetoleic acid, CH<sub>3</sub>(H<sub>2</sub>)<sub>9</sub>CH=CH(CH<sub>2</sub>)<sub>9</sub>COOH,  
 Erucic acid, CH<sub>3</sub>(CH<sub>2</sub>)<sub>7</sub>CH=CH(CH<sub>2</sub>)<sub>11</sub>COOH,  
 75 Nervonic acid, CH<sub>3</sub>(CH<sub>2</sub>)<sub>7</sub>CH=CH(CH<sub>2</sub>)<sub>13</sub>COOH,

all of which are obtainable by the hydrolysis of the corresponding natural esters.

It is readily observable that in these monoolefinic and polyolefinic  $R_dCOO-$  groups that (1) there is no terminal  $CH_2=C<$  structure, rather the terminal group is a  $CH_3-$  group, (2) the first double bond in the structure is removed from the oxygen atom of its esters, by at least 4 carbon atoms and by as many as 14 carbon atoms, and therefore are not activated by the ester structure, (3) the first double bonds are removed by at least 1 carbon atom from the terminal  $-CH_3$  group which is not an activating group, and there are 1 to 4  $-CH=CH-$  groups in the unsaturated portion of the acid molecule. In this regard they are similar to the  $R_dCH_2OH$  alcohol, and the  $R_d$  portion of both the  $R_dCH_2OH$  and  $R_dCOOH$  are identically defined.

For the purposes of this invention the pure individual  $R_dCOOH$  acids are not required although some of them have become available commercially in different degrees of purity. Mixtures of the acids, such as are obtained by the hydrolysis of vegetable, animal and marine oils and fats are satisfactory. Since such oils and fats are mixtures of various glycerides, the acids resulting from the hydrolysis of the ester groups correspond equivalently to the amounts of acid moiety present in the glyceride. Table 1 gives the percentage composition of the fatty acids in a number of drying oils, which on hydrolysis produce an equivalent amount of the corresponding acids and are useful in preparing the monomers suitable for the practice of this invention.

It will be noted in Table 1 that all of the oils have measurable amounts of compounds having one or more than one double bond in the fatty acid and therefore, the derived acids have a substantial amount of suitable mono- and poly-unsaturation suitable for the purposes of this invention. Palmitic and stearic acids are saturated acids, and if present in the mixture during esterification with a polyhydric alcohol,  $HO-Y-OH$ , also become converted to esters and copolymerize with the other monomers, lending flexibility and ductility to the polymerization product. Mixture of such acids are useful and the monomeric esters resulting from such mixtures are also contemplated in the practice of the invention.

As shown hereinabove, the radical,  $-Y-$ , is derived from polyols containing at least two hydroxyl groups, one hydroxyl group of which is used for bonding to the



moiety and at least one to the  $R_dCOO$ -moiety, so that the radical,  $-Y-$  derived from the polyol may be written as  $-Y-(OOCR_d)_p$ , wherein  $p$  represents an integer of one to five, and  $-Y-$  is a polyvalent radical containing 2 to 18 carbon atoms in which all the valencies not occupied by the one bond to  $CH_2=C(Ar)-$  and  $R_dCOO-$  bonds are occupied by  $R''$ ,  $OR''$ ,  $OCOR''$ , and  $-OH$  radicals. Illustrative polyols of the formula  $HO-Y-OH$ , as well as some cyclic oxides from which the  $-Y-$  groups are derived are,



The Class B esters are readily prepared by reacting an  $R_dCOOH$  acid compound with the suitable alcohol derivative of the



radicals as illustrated with vinylbenzyl alcohol,



An alternate method is to use the acid chloride in the presence of a hydrohalide acceptor,



The vinyl benzyl alcohol is illustrative of other alcohols which can be used, e.g.,



The Class C ethers are also readily prepared by reacting an  $R_dCH_2OH$  alcohol or a  $R_dCH_2X$  halide with a suitable halide or alcohol derivative of a



radical. These reactions may be illustrated in one case with vinyl benzyl chloride, thus



## 13

Instead of vinyl benzyl chloride, other halides such as



etc. may be used. The inverse reaction may also be used 10 as where the alcohol function is attached to the



radical, thus



in which the alcoholates are prepared from the alcohol and an alkali metal. Other alcohols which can be used as alcoholates with  $\text{R}_d\text{CH}_2\text{X}$  are,



The Class D hydrocarbons are best prepared through 30 the Grignard reaction, thus,



or



Thus it may be seen that a wide variety of monomers useful in the practice of this invention can be prepared by well-known and established reactions, and that the monomers can be defined as having the general structure



to which is attached an  $\text{R}_d$  radical through ether, esters or hydrocarbon linkages. Since these monomers contain one



group and at least one  $\text{R}_d$  group, they possess a multiplicity of polymerizable double bonds, of which the bond in the



group is very reactive, and at least one other



group in some cases four  $\text{CH}=\text{CH}$  groups.

Since in a polymerization, all of the ethylenic groups can participate, it would be expected that crosslinked, insoluble, infusible polymers are obtained from these monomers, and therefore a directed polymerization would be necessary to prepare soluble, fusible polymers and copolymers. When these monomers are polymerized by radical initiation, crosslinked gelled polymers result; and similar insoluble products are obtained with thermal polymerizations. When cationic initiators such as  $\text{BF}_3$ ,  $\text{AlCl}_3$ ,  $\text{H}_2\text{SO}_4$ ,  $\text{SnCl}_4$ ,  $\text{TiCl}_4$  etc. are used, insoluble, infusible products are likewise obtained.

However, I have discovered that useful linear, soluble polymers and copolymers are obtained when a base-

## 14

catalyzed polymerization is performed, such as in an anionic polymerization. By an anionic polymerization is meant a polymerization in which the propagation of the polymer chain occurs through a carbanion. This may be illustrated by rewriting the monomers,



15 wherein  $\text{R}_2$  represents  $\text{Ar}-\text{Z}$ , thus



etc., in which  $\text{Z}^{\oplus}$  is a positive counter ion, usually a metal, typically an alkali or alkaline earth metal. The propagation step is preceded by an initiating step; and initiation 25 may be brought about in a number of ways.

The anionic polymerization can be initiated by an alkali metal hydride such as  $\text{NaH}$ ,  $\text{LiH}$ ,  $\text{KH}$ ,  $\text{CsH}$ , including various complexes thereof, such as  $\text{LiAlH}_4$  etc. Designating such hydrides as  $\text{MH}$ , then the initiating step is



When an alkali metal alkyl is used, the initiating step 35 is given as



in which the cation  $\text{M}^{\delta+}$  represents  $\text{Li}$ ,  $\text{Na}$ ,  $\text{K}$ ,  $\text{Cs}$  etc. and the anion  $\text{R}^-$  represents methyl, ethyl, propyl, isopropyl, butyl, amyl, isoamyl, benzyl, triphenyl, methyl, phenyl, naphthyl, octyl, etc., preferably containing no 45 more than 12 carbon atoms in said anion. A few typical examples of  $\text{MR}$  are



50 allyl sodium, etc.

A Grignard reagent  $\text{RM}_g\text{X}$  can also be used to initiate an anionic polymerization, thus



Illustrative examples of  $\text{RM}_g\text{X}$ , wherein  $\text{R}$  is as defined above, and  $\text{X}$  is a halogen such as phenyl magnesium bromide, butyl magnesium bromide and chloride, vinyl magnesium bromide, allyl magnesium bromide, etc.

The free alkali metals can also be used to initiate polymerization, especially when the metal,  $\text{M}^{\circ}$ , gives up an electron to form an ion radical of the monomer, thus



70 The ion radicals couple to form a dianion, thus



75 as a step in the initiation mechanism.

## 15

A similar mechanism occurs in the anionic initiation using an alkali metal and naphthalene, anthracene,  $\alpha$ -methyl styrene tetramer, etc., as illustrated by naphthalene, thus



The alkali metals in liquid ammonia are also effective anionic polymerization initiators which may function in either of two ways, e.g., in the case of potassium, calcium, or sodium in liquid ammonia the resulting amide functions as the initiator, thus



then



In the case of lithium an ion radical is formed in the reaction which acts as the initiator, thus



where  $e^-$  is an electron, thus



In the ammonia amide series, the order of reactivity of the cations is given as



In a similar way anionic initiation may be brought about by ketyls which are the reaction products of an alkali or alkaline earth metal with a ketone such as benzophenone in ether, thus



The anionic polymerization is performed with the monomers of this invention, alone or in the presence of a liquid diluent, at temperatures ranging from about  $-80^\circ C$ . to  $80^\circ C$ . For most monomers the range of  $-40^\circ C$ . to  $60^\circ C$ . is satisfactory, but in general,  $-20^\circ C$ . to  $40^\circ C$ . is more practical.

The solvents, or diluents, when used, may be selected from the class of aliphatic and aromatic hydrocarbons, ketones, ethers and esters, such as butane, propane, hexane, heptane, octane, benzene, toluene, xylene, dimethyl ether, diethyl ether, dibutyl ether, tetrahydrofuran, dioxane, diphenyl ether, dibenzyl ether, dimethyl ethylene glycol ether, dibutyl ethylene glycol ether, diethyl diethylene glycol ether, etc. The diluent or solvent can also act to control the molecular weight of the polymerization

5

by solvalytic chain transfer with the anion when protonic solvents are used, thus



Anionic polymerizations are also referred to as base-catalyzed polymerizations. For economical use as coating compositions, it is wasteful as well as unnecessary to use homopolymers of the monomers of this invention, since the high activity of polymers having such an abundance of air-drying functions such as in

15



is not needed in most cases, although they can be used as such in castings for encapsulation or impregnation. In most applications, copolymers with other monomers are preferred, particularly after it was discovered that the air-drying property of these monomers is conferred on the copolymers, which may be dipolymers, tripolymers, etc., depending on the number of additional monomers used as well as on the identity of the

25



monomer. A typical case is where the monomer is prepared from  $R_dCOOH$  acids or  $R_dCH_2OH$  alcohols derived from natural oils such as linseed or oiticica oil which contains 5 different compounds, as shown in Table 1.

In many cases, especially with the pure monomers derived from pure alcohols or acids, in which  $R_d$  contains four  $-HC=CH-$  group, copolymers containing 0.5 to 1% of these monomers are useful, but to achieve better air drying rates, copolymers containing at least 5% are preferable. When the  $R_d$  group contains fewer  $-CH=CH-$  groups, 10 to 20% of the monomer in the copolymer is advantageous. When the monomer is produced from alcohols or acids having a high percentage of saturated higher fatty acids or alcohols, then 50-80% or more are preferable. Accordingly, depending on the end product

desired and the use to which it is to be put, copolymers containing as little as 0.5% are useful. When less than 0.5%, such as 0.1% is used, then drying is greatly reduced, but, in this case, a noticeable plasticizer effect is evident and in this aspect these copolymers are useful and valuable. Obviously, those copolymers having more than 0.1% show higher internal plasticization, and when this particular property is desired, it is achieved by the practice of this invention. Accordingly, a wide range of compositions can be made by copolymerizing these monomers with one or more other monomers containing a vinyl,  $CH_2=CH-$  group, a vinylidene  $CH_2=C<$  group, or a vinylene  $-CH=CH-$  group.

Illustrative examples of other monomers containing such groups are the acrylic esters such as methyl acrylate, ethyl acrylate, propyl acrylate, butyl acrylate, hexyl acrylate, phenyl acrylate, benzyl acrylate, methyl- $\alpha$ -chloroacrylate, etc.; the methacrylic esters such as methyl methacrylate, ethyl methacrylate, propyl methacrylate, methylallyl methacrylate, etc.; the vinyl esters such as vinyl chloride, vinyl acetate, vinyl stearate, vinyl benzoate, vinyl methyl phthalate, vinyl ethyl succinate, etc.; the polymerizable amides and nitriles such as N-dimethyl acrylamide, N-diethyl methacrylamide, acrylonitrile, methacrylonitrile, etc.; the alkenyl aryl compounds such as styrene,  $\alpha$ -methyl styrene, p-methyl styrene,  $\alpha$ -methyl styrene, the chlorostyrene, vinyl methoxy benzene, diallyl benzene, etc.; the vinylidene compounds such as vinylidene cyanide, methylene malonic esters, etc.; vinylene compounds such as vinylene carbonates, and the maleic esters, especially the maleic diesters of the lower alcohols;

75

the itaconic compounds such as itaconic anhydride, the itaconic esters of the lower and higher aliphatic alcohols; the dienes such as butadiene, isoprene, and the like.

The proportion of the new monomers in copolymers with other monomers will depend, in accordance with the accepted principles of copolymerization, on the reactivity and selectivity constants of the comonomers used in preparing the copolymer, the ratio of the monomers used and the extent of conversion. However, by selecting appropriate conditions for the copolymerization copolymers using the new monomers of this invention, can be made to contain effective and small amounts of these new monomers, for example, of the order of from 0.1% to 0.5% to very high amounts of the order of 99.5% to 99.9% in the final copolymer products.

In anionic copolymerizations, the copolymerization parameter,  $r_1$  and  $r_2$ , are sometimes influenced by the solvent is one is used, for example, when a 50% benzene solution of a mixture of 90% vinylacetate and 10% of  $\text{CH}_2=\text{CHC}_6\text{H}_4\text{COOC}_{17}\text{H}_{33}$  with Na as an initiator, is polymerized at 30° C., less than 2% of the benzoate feed is found in the copolymer, whereas when the polymerization is performed in bulk without a solvent, about 27% of the benzoate is found in the copolymer. On the other hand, when the benzoate is copolymerized with ethyl acrylate or styrene, 100% of the monomer is found in the copolymer whether the copolymerization is performed in bulk or in a solution. Thus, while it is seen that same monomers polymerize less readily with the monomers of this invention, the resulting copolymers may still be used as air convertible compositions. The comonomers give corresponding repeating units such as



from styrene,



from methyl acrylates, etc.

The polymers and copolymers of this invention may be used as prepared or blended or compounded with other polymers and ingredients. When prepared and obtained in a viscous liquid form they may be used without solvent for casting, laminating and impregnating uses, or, to lower the resin content, or to control or regulate the viscosity, they may be diluted with solvents, or emulsified with water and used in the latex form. When obtained as soft resins, they can be diluted or emulsified, or used as melts to coat or impregnate substrates. When prepared as hard polymers they can be used in solution, or in emulsion, or in dispersions, or as dip-melts, or spray-melts, or fluidized-melts, etc. The polymers and copolymers can be blended with other drying and semi-drying or non-drying oils with or without a solvent; or they can, in a similar way, be blended or reacted with alkyd resin modified with drying or demi-drying oil acids, oil soluble phenolic resin, oil modified phenolic resins, etc. They can be used as blends with other film forming polymers, such as nitro-cellulose, polyvinyl acetate, polymethyl methacrylate, polyvinyl chloride and its copolymers, polystyrene and its copolymers, especially the butadiene copolymers; the blends being achieved either in solution or in emulsion, or without solvents. The polymers and copolymers of this invention, including blends with other polymers, can be converted to varnishes, paints, enamels and impregnants in the usual way and can be mixed with dyes, solvents, pigments, lubricants, stabilizers, etc; as is common in the coating arts. As such, they are useful not only as direct coatings but are particularly satisfactory for the preparation of oil cloths, electrical oil-cloth-insulating tapes, rain coats, linoleums, inks, etc.; when fabrics, paper, cloth, cork, mica, etc. are coated or impregnated with these compositions.

When properly prepared the polymers and copolymers

of this invention are substantially colorless or nearly so if the monomer is colorless, and the dried films have excellent resistance to yellowing compared to films prepared from drying oils or drying oil-modified alkyd resins and similar compositions. Also, those polymers in which the  $\text{R}_d$  group is bonded to the



radical through ether or hydrocarbon linkages, are extremely resistant to acids and alkali which readily hydrolyze alkyd-type resins.

The following examples illustrate the practice of this invention and are used by way of illustration and not intended in any way to limit the scope of this invention nor the manner in which it can be practiced. All parts and percentages are parts and percentages by weight, unless otherwise specified.

*Example I*

20 Two hundred sixty-six parts of linoleyl alcohol, 0.1 part of tertiary butyl catechol, and 185 parts of tributyl amine are added to 1000 parts of diethyl ether in a suitable container equipped with stirrer, reflux condenser and heating and cooling means; the mixture is blanketed with nitrogen gas through an inlet. To this mixture is added over a period of 2 hours at 20° C., 166.5 parts of vinyl benzoyl chloride in 200 parts of ether, following which the temperature is raised to 30-35° C. for 1 hour. The mixture is then washed with dilute hydrochloric acid, then with water to remove trimethyl amine hydrochloride, followed by washing with dilute aqueous sodium carbonate and again with water until neutral. The resulting ether solution of the ester,  $\text{CH}_2=\text{CHC}_6\text{H}_4\text{COOC}_{18}\text{H}_{33}$  is dried over anhydrous  $\text{Na}_2\text{CO}_3$ , decolorized with active carbon and filtered. The monomer is isolated by distilling off the ether at reduced pressure leaving the monomer. Analysis for carbon and hydrogen gives values of 81.79% C. and 10.01% H., which are in good agreement with the theoretical values of the compound. The monomer is polymerizable in pure form or in the ether solution prior to isolation.

When 268 parts of oleyl alcohol are used instead of the linoleyl alcohol, then the corresponding ester (a)



is obtained, whereas when 264 parts of linolenyl alcohol is used, then the corresponding ester, (b)



50 is obtained, which on analysis for carbon and hydrogen gives values of 81.54% C and 10.78% H for (a) and 81.9% C and 9.88% H for (b); which are in close agreement with the theoretical values for these compounds. Similarly, when 180.5 parts of



55 is used instead of vinyl benzoyl chloride in this procedure, then the corresponding esters,



and



60 are obtained.

*Example II*

One hundred sixty-two parts of methyl p-vinyl-benzoate, 133 parts of linoleyl alcohol, 0.5 part tertiary butyl catechol, and 1.5 parts of sodium methylate are heated to 80-100° C. and the methyl alcohol resulting from trans-esterification is removed continuously in a distillation column until no more methyl alcohol is released. The unreacted sodium is then neutralized with gaseous HCl,

## 19

and the NaCl product removed by filtration. The excess methyl p-vinyl-benzoate is removed by distillation, leaving the crude ester,  $\text{CH}_2=\text{CHC}_6\text{H}_4\text{COOC}_{18}\text{H}_{33}$ . This is purified by treatment with active carbon and distillation as in the procedure of Example I. The crude ester is also polymerized as such.

## Example III

Two hundred seventy-six parts of the anhydride,



and 266 parts of linoleyl alcohol and 185 parts of tributyl amine are reacted and then isolated according to the procedure of Example I, and the benzoate ester identical to that of Examples I and II is obtained.

## Example IV

A commercial product comprising unsaturated fatty alcohols having an iodine value of 125, and a hydroxyl value of 210, containing the following alcohols in the proportions

|                      | Percent           |
|----------------------|-------------------|
| Linoleyl alcohol     | 53                |
| Linolenyl alcohol    | 8                 |
| Oleyl alcohol        | 25                |
|                      | (Unsaturated 86%) |
| Cetyl alcohol        | 8                 |
| Stearyl alcohol      | 5                 |
| Arachidyl and others | 1                 |
|                      | (Saturated 14%)   |

is substituted for the linoleyl alcohol of Examples I and II. Mixed esters corresponding to the formula



are obtained, in which  $\text{R}_{dx}$ , although embraced by  $\text{R}_d$ , is used to represent specifically the mixed hydrocarbon groups in the mixed alcohol as shown above.

## Example V

Example I is repeated using a mixture of unsaturated fatty alcohols having an iodine value of 170, a hydroxyl value of 210, and containing the approximate composition

|                   | Percent           |
|-------------------|-------------------|
| Linoleyl alcohol  | 17                |
| Linolenyl alcohol | 51                |
| Oleyl alcohol     | 21                |
|                   | (Unsaturated 89%) |
| Cetyl alcohol     | 6                 |
| Stearyl alcohol   | 5                 |
|                   | (Saturated 11%)   |

The resultant mixed ester,  $\text{CH}_2=\text{CHC}_6\text{H}_4\text{COOR}_{dx}$ , is polymerizable.

## Example VI

Example IV is repeated using a mixture of unsaturated alcohols comprising oleyl alcohol in the major amounts, and linoleyl, linolenyl, cetyl, and stearyl in the minor amounts with an iodine value of about 90 (known as Adol 85 of Archer-Daniels-Midland), and there is obtained the mixed esters corresponding to the formula



## Example VII

Under an inert nitrogen atmosphere, to each of fifty parts of linoleyl vinyl benzoate monomer of Example I in five separate reaction vessels is added 50 parts of anhydrous benzene and (1) 0.1, (2) 0.25, (3) 0.50, (4) 1.00, and (5) 1.5 parts of micronized sodium respectively at 25° C., and within about an hour, the solution, due to the presence of styryl-type anions, becomes bluish green, with the dissolution of the sodium. The mixture is agi-

## 20

tated for 48 hours at 25° C. and anhydrous HCl gas is then passed into the mixture to remove the color, after which the solid NaCl is removed from the solution by filtration. The resulting solutions of polymer in benzene may be used as such or the polymer may be isolated by removing the solvent by distillation at 15 mm. pressure. The yield of residue is substantially quantitative and all of them are very viscous thick products. The polymer prepared with 0.1 part (0.2% based on the monomer) of sodium initiator is the most viscous and the polymer prepared with 1.5 parts of sodium (3% on the monomer) is the least viscous, and the other polymers prepared with intermediate sodium concentrations have viscosities between these two extremes.

## Example VIII

Example VII is repeated in the absence of benzene solvent but at 30° C. for 72 hours to effect better dissolution of the sodium and polymers similar to those of Example VII are obtained.

## Example IX

Three hundred twenty-four parts of freshly distilled hydroxyethyl linoleate,  $\text{C}_{17}\text{H}_{31}\text{COOCH}_2\text{CH}_2\text{OH}$ , 0.1 part of tertiary butyl catechol, and 185 parts of tributyl amine are added to 1000 parts of diethyl ether in a suitable container equipped with stirrer, reflux condenser and heating and cooling means; the mixture is blanketed with nitrogen gas through an inlet. To this mixture is added over a period of 2 hours at 20° C., 166.5 parts of vinylbenzoyl chloride in 200 parts of ether, following which the temperature is raised to 30-35° C. for 1 hour. The mixture is then washed with dilute hydrochloric acid, then water to remove trimethyl amine hydrochloride, followed by washing with dilute aqueous sodium carbonate and again with water until neutral. The resulting ether solution of the ester is treated according to the procedure of Example I, and there is isolated the monomer



When 326 parts of hydroxyethyl oleate are used instead of the linoleate, then the corresponding ester



is obtained. When 322 parts of hydroxyethyl linolenate is used, then the ester



is obtained, which on analysis gives values of 76.91% C and 8.79 H, which are in good agreement with the theoretical values for the compounds. These monomers are polymerized with similar results by the procedure of Example VII using 0.05% by weight of sodium.

## Example X

Three hundred twenty (320) parts of a redistilled commercial product comprising unsaturated fatty acids derived from soyabean oil and containing the following acids in the proportions

|                | Percent           |
|----------------|-------------------|
| Linoleic acid  | 53                |
| Linolenic acid | 7                 |
| Oelic acid     | 25                |
|                | (Unsaturated 85%) |

|               |   |
|---------------|---|
| Palmitic acid | 8 |
| Stearic acid  | 6 |
| Other acids   | 1 |

(Saturated 15%)

are reacted at 150° C. with 44 parts of ethylene oxide in a pressure autoclave at 110° C. in the presence of 1 part of KOH during the course of two hours. The reaction product is cooled, neutralized with acetic acid and flash distilled at 2 mm. pressure. The mixed hydroxylalkyl es-

21

ters are substituted for the hydroxyethyl linolenate of Example IX, and esters corresponding to the formula



are obtained, in which  $\text{R}_{\text{dx}}$  represents the mixed hydrocarbon groups in the mixed acids.

*Example XI*

Example X is repeated using a mixture of commercial unsaturated fatty acids having an iodine value of 170, containing the approximate composition

|                | Percent           |
|----------------|-------------------|
| Linoleic acid  | 18                |
| Linolenic acid | 48                |
| Oleic acid     | 22                |
|                | (Unsaturated 88%) |
| Palmitic acid  | 7                 |
| Stearic acid   | 5                 |
|                | (Saturated 12%)   |

resulting in the mixed esters,



*Example XII*

Example X is repeated using a mixture of unsaturated acids comprising oleic acid in the major amounts, and linoleic, linolenic, palmitic, and stearic acids in the minor amounts with an iodine value of about 90, and there is obtained the mixed esters corresponding to the formula,  $\text{CH}_2=\text{CHC}_6\text{H}_4\text{COOCH}_2\text{CH}_2\text{OOCR}_{\text{dx}}$ .

*Example XIII*

Under an inert nitrogen atmosphere, to each of fifty parts of the



monomer of Example X in five separate reaction vessels is added 50 parts of anhydrous benzene and (1) 0.25, (2) 0.50, (3) 1.00, (4) 1.5, and (5) 2.0 parts of micronized sodium respectively at 25° C. Within an hour, the solution, due to the presence of styryl-type anions, becomes greenish, with the dissolution of the sodium. Each mixture is agitated for 48 hours at 25° C., then anhydrous HCl gas is passed into the mixture to remove the color, and the solid NaCl is thereafter removed from the solution by filtration. The resulting solutions of polymer in benzene may be used as such or the polymer may be isolated by removing the solvent by distillation at 15 mm. pressure. The yield of residue in each case is substantially quantitative. All are very viscous thick products. The polymer prepared with 0.25 part (0.5% based on the monomer) of sodium initiator is the most viscous, and the polymer prepared with 2 parts of sodium (4% on the monomer) is the least viscous. The other polymers prepared with intermediate sodium concentrations have viscosities between these two extremes.

*Example XIV*

Example XIII is repeated in the absence of benzene solvent but at 30° C. for 72 hours to effect better dissolution of the sodium and polymers similar to those of Example XIII are obtained.

*Example XV*

Example I is repeated using instead of



an equivalent amount of the following acid chlorides prepared from the corresponding acids and  $\text{SOCl}_2$ :



22

and the corresponding monomers:



are obtained, which are polymerized by the procedure of Example VII.

*Example XVI*

Example X is repeated using 132 parts of ethylene oxide instead of 44 parts and there is obtained the monomer  $\text{CH}_2=\text{CHC}_6\text{H}_4\text{CO}(\text{OCH}_2\text{CH}_2)_3\text{OOCR}_{\text{dx}}$ , and when 174 parts of propylene oxide is used, there is obtained the monomer



both of which are readily polymerized by the procedure of Example VII.

*Example XVII*

25 The mixed alcohols of Example IV are reacted with 5 mol equivalent of ethylene oxide by the procedure of Example X and converted to esters by the procedure of Example I and the mixed esters corresponding to the formula  $\text{CH}_2=\text{CHC}_6\text{H}_4\text{CO}(\text{OCH}_2\text{CH}_2)_5\text{OCH}_2\text{R}_{\text{dx}}$ , are obtained which are shown to be polymerized by the procedure of Example VII.

*Example XVIII*

35 The procedure of Example I is repeated using 164 parts of (vinylphenoxy)ethyl alcohol,



300.5 parts of  $\text{C}_{17}\text{H}_{31}\text{COCl}$  and 185 parts of butyl amine, and there is obtained the monomer



When 298.5 parts of  $\text{C}_{17}\text{H}_{31}\text{COCl}$  and 296.5 parts of  $\text{C}_{17}\text{H}_{29}\text{COCl}$  are used instead of the oleyl chloride, the esters,  $\text{CH}_2=\text{CHC}_6\text{H}_4\text{OCCH}_2\text{CH}_2\text{OCOC}_{17}\text{H}_{31}$  and



45 respectively are obtained.

*Example XIX*

Example XVIII is repeated using instead of



with  $\text{C}_{17}\text{H}_{31}\text{COCl}$  the following alcohols,

55 178 parts of  $\text{CH}_2=\overset{\text{CH}_3}{\text{C}}\text{C}_6\text{H}_4\text{OCH}_2\text{CH}_2\text{OH}$   
208 parts of  $\text{CH}_2=\text{CHC}_6\text{H}_4(\text{OCH}_2\text{CH}_2)_2\text{OH}$   
236 parts of  $\text{CH}_2=\text{CHC}_6\text{H}_4(\text{OCH}_2\text{CHCH}_3)_2\text{OH}$   
134 parts of  $\text{CH}_2=\text{CHC}_6\text{H}_4\text{CH}_2\text{OH}$   
234 parts of  $\text{CH}_2=\text{CHC}_6\text{H}_4\text{CH}_2\text{O}(\text{CH}_2)_6\text{OH}$   
238 parts of  $\text{CH}_2=\text{CHC}_6\text{H}_4\text{OCH}_2\text{COOCH}_2\text{CH}_2\text{CH}_2\text{OH}$   
60 there are obtained respectively the corresponding monomers



70 When this procedure is repeated with  $\text{C}_{17}\text{H}_{31}\text{COCl}$  and  $\text{C}_{17}\text{H}_{29}\text{COCl}$ , then the corresponding esters are obtained.

*Example XX*

75 The procedure of Example XIX is repeated with the acid chlorides of Example XI, and the corresponding

## 23

monomers having a  $R_{dx}COO-$  ester structure are obtained.

## Example XXI

Example XVIII is repeated using 236 parts of



(prepared by heating 60 parts of  $\text{CH}_3\text{COOH}$  and 176 parts of



instead of  $\text{CH}_2=\text{CHC}_6\text{H}_4\text{OCH}_2\text{CH}_2\text{OH}$ ). There are obtained



and



When 146 parts of divinyl benzene monoxide,



is used in this procedure, then



and



are obtained respectively.

When acids other than acetic acid are used with the starting epoxide, such as benzoic acid, etc., then the corresponding derivative is obtained, as illustrated with the oleate,



## Example XXII

A mixture of 120 parts of vinyl phenol



23 parts of  $\text{NaOH}$  in  $\text{C}_2\text{H}_5\text{OCH}_2\text{CH}_2\text{OC}_2\text{H}_5$  are refluxed with 272.5 parts of  $\text{C}_{17}\text{H}_{33}\text{Cl}$  for 12 hours. Then the solvent is removed under a reduced pressure of 15 mm., 500 parts of ether are added and the solution filtered to remove salt. The filtrate is washed with water, dried over anhydrous  $\text{Na}_2\text{CO}_3$ , filtered, then decolorized with charcoal, and the ether removed by evaporation. There is obtained the monomer  $\text{CH}_2=\text{CHC}_6\text{H}_4\text{OC}_{17}\text{H}_{33}$ .

When for the alkene chloride there is used 270.5 parts of  $\text{C}_{17}\text{H}_{31}\text{Cl}$  or 268.5 parts of  $\text{C}_{10}\text{H}_{29}\text{Cl}$  there are obtained  $\text{CH}_2=\text{CHC}_6\text{H}_4\text{OC}_{17}\text{H}_{31}$  and  $\text{CH}_2=\text{CHC}_6\text{H}_4\text{OC}_{17}\text{H}_{29}$  respectively.

## Example XXIII

The procedure of Example XXII is repeated using 288 parts of  $\text{C}_{18}\text{H}_{33}\text{ONa}$  and 142.5 parts of



and there is obtained the monomer



## Example XXIV

Example XXIII is repeated using 226.5 parts of



## 24

(from  $\text{CH}_2=\text{CHC}_6\text{H}_4\text{ONa}$  and  $\text{ClCH}_2\text{CH}_2\text{OCH}_2\text{CH}_2\text{Cl}$ ), and there is obtained



## Example XXV

In 1000 parts tetrahydrofuran, a Grignard reaction is performed with 142.5 parts of  $\text{CH}_2=\text{CHC}_6\text{H}_4\text{CH}_2\text{Cl}$  and 292.8 parts of  $\text{C}_{17}\text{H}_{29}\text{MgCl}$  (from  $\text{C}_{17}\text{H}_{29}\text{Cl} + \text{Mg}$ ), and the monomer,  $\text{CH}_2=\text{CHC}_6\text{H}_4\text{CH}_2\text{C}_{17}\text{H}_{29}$  is isolated by evaporation of the tetrahydrofuran by the procedure of Example XXII.

## Example XXVI

Example I is repeated using 620 parts of glyceryl dioleate instead of 266 parts of linoleyl alcohol and the monomer  $\text{CH}_2=\text{CHC}_6\text{H}_4\text{COOC}_3\text{H}_5(\text{OCOC}_{17}\text{H}_{33})_2$  is isolated by evaporation of the dry ether solution after treatment with activated carbon.

## Example XXVII

The procedure of Example I is repeated using 143 parts of  $\text{CH}_2=\text{CHC}_6\text{H}_4\text{CH}_2\text{N}(\text{CH}_2\text{COCl})_2$  instead of the vinyl benzoyl chloride and there are obtained the monomers  $\text{CH}_2=\text{CHC}_6\text{H}_4\text{CH}_2\text{N}(\text{CH}_2\text{COOC}_{18}\text{H}_{33})_2$



and  $\text{CH}_2=\text{CHC}_6\text{H}_4\text{CH}_2\text{N}(\text{CH}_2\text{COOC}_{18}\text{H}_{31})_2$  respectively.

When the acid chloride of the N-(ar-vinylbenzyl)-imidodiacetic acid of this example is replaced by other vinylphenyl aliphatic aminocarboxylic acids given in U.S. Patents 2,840,603; 2,875,162; 2,888,441; 2,910,445, then the corresponding monomer esters are obtained.

## Example XXVIII

In an inert atmosphere, a mixture of 80 parts of styrene and 20 parts of linoleyl vinyl benzoate of Example I are added to 200 parts of anhydrous benzene, and to this solution is added 1.1 parts of micronized sodium in 1.1 parts of kerosene at 25° C. and allowed to react for 24 hours with slow agitation. The mixture is then neutralized with 2.8 parts of glacial acetic acid and the solution filtered to remove precipitated salts. The copolymer yield is almost quantitative, and the intrinsic viscosity is 0.124. Titration of the copolymer with bromine for unsaturation shows that the copolymer contains about 20% of linoleyl vinyl benzoate in the copolymer.

## Example XXIX

The procedure of Example XXVIII is repeated twice using instead of 20 parts of linoleyl vinyl benzoate, 20 parts respectively of oleyl vinyl benzoate and linolenyl vinyl benzoate, and the corresponding copolymers of styrene, respectively, of approximately the same molecular weight, are obtained. After filtration of the benzene solutions, they are evaporated at 20° C. at 10 mm. and almost quantitative yields of copolymers are obtained, with only slight trace of yellow color. The copolymers are soluble in common solvents, such as the ketones, toluene, esters and halogenated hydrocarbons.

## EXAMPLE XXX

The procedure of Example XXVIII is repeated using 93 parts of styrene and 7 parts of the ester,  $\text{CH}_2=\text{CHC}_6\text{H}_4\text{COOR}_{dx}$  of Example IV and 2 parts of BuLi (as a 30% solution in ethyl ether) are added under a nitrogen atmosphere to 200 parts of anhydrous benzene at 0° C. for 15 hours, then allowed to heat to room temperature during a period of 3 hours, following which 3 parts of glacial acetic acid is added to neutralize the lithium and the solution filtered. The polymer solution is then poured into methanol and 96 parts of solid, precipitated copolymer is obtained which, on analysis, indicates a copolymer of approximately 93.1% styrene and 6.9% of the  $\text{CH}_2=\text{CHC}_6\text{H}_4\text{COOR}_{dx}$  monomer. In a

similar manner a 50-50 copolymer is prepared from equal parts of styrene and the ester of Example IV.

*Example XXXI*

The procedure of Example XXVIII is repeated using 85 parts of butyl methacrylate, 15 parts of the ester,  $\text{CH}_2=\text{CHC}_6\text{H}_4\text{COOR}_{\text{d}}$ , of Example IV and 5 parts of finely divided sodium hydride in a sealed reactor which had been degassed and blanketed with deoxygenated nitrogen and the polymerization conducted at  $-5^{\circ}\text{C}$ . to  $5^{\circ}\text{C}$ . for 24 hours. The reaction product is then neutralized with 10 parts of anhydrous acetic acid, filtered and then concentrated by distillation at 10 mm. at  $25^{\circ}\text{C}$ ., leaving 96.3 parts of a rubbery polymer product.

*Example XXXII*

The procedure of Example XXVIII is repeated using 65 parts styrene, 25 parts of methyl acrylate and 10 parts of the monomer,  $\text{CH}_2=\text{CHC}_6\text{H}_4\text{COOR}_{\text{d}}$  of Example VI as the monomer feed and the corresponding tripolymer obtained.

*Example XXXIII*

To ten parts each of the five polymers of Example VII in twenty parts of benzene respectively is added 0.1 part of commercial 10% drier solution containing lead, manganese and cobalt in the approximate ratio of 9.6:1:1.8 as naphthenates. Films of the resultant compositions are prepared on glass plates and the solvent allowed to evaporate at room temperature. On evaporation of the solvent, the residue varies from viscous oily coatings to tacky films, are initially soluble in benzene and acetone, but after seven or eight hours, become converted to dry, substantially colorless, elastic, tough films, insoluble in benzene, acetone and dioxane. When the metallic drier is omitted from the formulation, dry but less elastic films are obtained in 24-36 hours.

*Example XXXIV*

The procedure of Example XXXIII is repeated with (1) the three polymers of Example IX; (2) the styrene copolymers of Example XXVIII; (3) the styrene copolymer of Example XXIX; (4) the styrene mixed drying oil alcohols-vinyl benzoate copolymer of Example XXX; (5) the butyl methacrylate-copolymer of Example XXXI; and (6) the terpolymer of Example XXXII. In all cases the coatings become converted to benzene-insoluble films in 8-12 hours at room temperature, when the drier is used.

*Example XXXV*

Linseed oil is heat polymerized at  $290^{\circ}\text{C}$ . under an inert atmosphere for 12 hours. Then the experiment is repeated using a mixture of 90% by weight of linseed oil and 10% by weight of the polymer (2) of Example VII. The viscosities of the stand-oil and polymer-modified stand-oil are compared in Table 2.

TABLE 2

| Time in hours | Viscosity of oil in Process | Viscosity of Oil plus polymer |
|---------------|-----------------------------|-------------------------------|
| 1             | 1.15                        | 3.8                           |
| 2             | 1.59                        | 28.6                          |
| 4             | 3.5                         | 71.0                          |
| 6             | 9.2                         | 152.8                         |
| 8             | 24.0                        | 205.4                         |
| 10            | 82.0                        | 392.6                         |
| 12            | 196.0                       | -----                         |
| 16            | 390.0                       | -----                         |

It will be noted that the addition of polymer to the oil causes a more rapid increase in the viscosity of the resulting stand-oil, and that at least 16 hours of heating are required by the unmodified oil to attain a viscosity equal to about ten hours heating of the polymer-modified oil. The same improvement in a reduction of the time required

to prepare stand oils from tung, perilla, oiticica, corn, hempseed, safflower, sandal seed and sunflower oil is observed when the polymers of this invention are added to the oil before heat treatment. Depending on the oil, the modified stand oil is prepared at temperatures varying from  $240^{\circ}\text{C}$ . to  $310^{\circ}\text{C}$ . and for periods of time varying from 1 hour to 12 hours, a factor which is also controlled by the amount of polymer added to the oil, and a reduction in the heating time is noted when the other polymers of Examples VII, VIII, IX, and XXVIII to XXXII are added to oil before or during the heat processing. The modified stand oils can be formulated into varnishes by dilution with solvents to which is added metallic driers, or they may be emulsified after drier addition and used in emulsion form.

*Example XXXVI*

To fifty parts of a long oil glyceryl phthalate alkyd resin containing 55% of combined linseed oil fatty acids in toluene is added 25 parts of a 50% solution in toluene of the polymer of Example XXXI and the drier content adjusted to 0.1% of metal content on the basis of polymer content. Films of this varnish dry in 2.5 hours whereas films prepared from this alkyd resin are not dry in 5.5 hours. A marked improvement in drying time is also shown when the polymers of Examples VII to IX, XXVIII to XXX, and XXXII are added in various amounts to a long oil glyceryl phthalate alkyd resin; and an even greater improvement is noted when these polymers are added to a short-oil alkyd resin containing about 40% of combined linseed oil fatty acids.

*Example XXXVII*

Linseed oil of specific gravity 0.9290, and containing 0.05% soluble lead salts and 0.08% soluble manganese salt, is heated to  $80^{\circ}\text{C}$ . while a stream of air is blown through it for 20 hours. A "boiled oil" of gravity 0.940 is thus obtained. When the process is repeated with a mixture of the same oil containing 10% of polymer (2) of Example VII, a boiled oil of the same gravity is obtained in 14 hours.

*Example XXXVIII*

To 10 parts of the polymer (2) of Example VII is added 6 parts of solid para-phenyl phenol-formaldehyde resins (known commercially as Bakelite-BR 254). The mixture is heated to  $220^{\circ}\text{C}$ . until a clear melt results when a drop is removed and placed on a glass plate. Then the product is dissolved in 35 parts of a solvent mixture of a ratio 2 parts of white spirits to 1 part of toluene, containing 0.1 part of commercial metal driers per part of the polymer. A film cast from this solution dries to a tack-free glassy, water-resistant film in 2-3 hours.

Similar good results are obtained when tertiary butyl phenol-formaldehyde resin is used instead of the phenyl-phenol resin.

*Example XXXIX*

To each of the three monomers of Example I corresponding to the formula



is added 1.5% by weight of benzoyl peroxide and the mixture heated at  $80-85^{\circ}\text{C}$ . No noticeable polymerization occurs in 6-8 hours but in 24-48 hours, benzene-insoluble, crosslinked gels are obtained.

*Example XL*

To a mixture of 90 parts of methyl methacrylate and 10 parts of the linoleyl vinyl benzoate is added 1 part of benzoyl peroxide and the mixture heated to  $80-85^{\circ}\text{C}$ . A benzene and acetone insoluble copolymer is obtained upon maintaining this temperature for 24 hours. Similar

results are obtained when the other two monomers of Example I are used instead of the linoleyl derivative.

*Example XLI*

To a mixture of 80 parts of styrene and 20 parts of linoleyl vinyl benzoate is added 0.3 part of  $\text{BF}_3$  at room temperature. A dark brownish mass, insoluble in benzene, is obtained.

*Example XLII*

To each of 100 parts of oleyl alcohol, linoleyl alcohol, and linoleyl alcohol is added 0.1 part of the drier of Example XXIII. Glass plates are coated with the respective mixtures. No drying occurs at room temperature in 6 days.

*Example XLIII*

To 100 parts of linoleyl acetate (prepared from acetic anhydride and linoleyl alcohol) is added 0.1 part of the drier of Example XXIII, and a glass plate is coated with the mixture as in Example XLII. No drying is observed in 6 days at room temperature.

*Example XLIV*

To 400 parts of anhydrous liquid ammonia at  $-77^\circ \text{C}$ . is added 0.1 part of sodium with the formation of a blue color indicating  $\text{NaNH}_2$  had formed and then is added a mixture of 18 parts of methyl methacrylate and 2 parts of linoleyl vinyl-benzoate to form a solid copolymer which is removed by filtration. The product is washed with 50-50 methyl alcohol-water mixture containing 3 parts HCl, followed by washing twice with a 50-50 methyl alcohol-water mixture, and then dried in vacuo to constant weight. A 95.2% yield of polymer is obtained.

*Example XLV*

A flat enamel is prepared according to standard procedures in the painting art containing 55% pigment and 45% vehicle in the following proportions.

| Total pigment 55% comprising:                                             | Percent |
|---------------------------------------------------------------------------|---------|
| Titanium pigment                                                          | 57.2    |
| Calcium carbonate                                                         | 36.0    |
| Diatomaceous silica                                                       | 4.8     |
| Zinc stearate                                                             | 2.0     |
| Total vehicle 45% comprising:                                             |         |
| Polymer Example XLIII                                                     | 20.0    |
| Polymer stand-oil of 395 viscosity of Example XXXV                        | 5.2     |
| Solvent (50-50 mineral spirits-toluene) containing 0.15 part metal driers | 74.8    |

A sized plaster surface is coated with this paint which dries in about three hours to give a very white satin finish with excellent water resistance that can be re-washed repeatedly.

*Example XLVI*

A commercial acrylic latex paint is applied (without first applying the sizing undercoat recommended when a latex is applied over oil-type paints) to wood previously coated with a drying oil-alkyd type paint and aged for at least 3 months. This new coating is allowed to air-dry for 24 hours and then exposed to weathering. To another part of the same acrylic latex is added 5% by weight of the copolymer of Example XXXI (previously emulsified as a 40% emulsion in water with dodecylbenzene sodium sulfonate) and applied in the same way as the unmodified acrylic latex. At the end of six months, peeling and blistering is observed in the film with the commercial latex, whereas the modified latex coating is continuous and intact. In a similar manner vinyl acetate and styrene-butadiene latices can be modified by the addition of the polymers of this invention to improve their properties.

*Example XLVII*

A mixture of 70 parts of asphaltic bitumen (M.P. 90°

C.) and 30 parts of polymer (2) of Example VII are heated at  $100^\circ \text{C}$ . for 15 minutes, then diluted with 70 parts of solvent mixture containing 80% white gasoline and 20% benzene and 0.03 part of metallic driers.

This solution is used to coat tin plate and allow to dry for 6 days. A similar solution of the asphaltic bitumen is prepared without including the polymer of Example VII and air dried for a similar period of time. When both plates are placed in an oven and the temperature raised to  $95^\circ \text{C}$ ., the coating not containing polymer sags and flows, whereas the solution containing the polymer does not sag or flow. Mixtures of asphaltenes of this type with the polymers of this invention, are particularly suitable for the preparation of gutter paint, rust proofing and water resistant coating for underground pipes of all kinds, including iron, brass, copper, and for exposed metal, ceramic, clay, wood, wall board, concrete and stone surfaces, as well as for the preparation of asphalt shingles, roofing paper, etc. Instead of the asphaltic bitumen, other bitumens such as blown asphaltic bitumens, stearine pitches, Grahamite (an asphaltum from Virginia and Oklahoma), Gilsonite (an asphaltum from Utah), coal tar pitches, etc., can also be modified by the polymers of this invention to improve their flow properties.

*Example XLVIII*

A mixture of 320 parts of linoleyl vinyl-benzoate and 11.5 parts of sodium are reacted at  $50^\circ \text{C}$ . according to the procedure of Example VII and the product isolated. Molecular weight determinations indicate that the product is a dimer. To 100 parts of the dimer is added one part of the drier of Example XVIII and a film prepared on a glass plate therefrom dries in 6-7 hours.

*Example XLIX*

To 30 parts of polymer (1) of Example VII is added 1.5 parts of sodium dioctyl sulfosuccinate and the mixture heated with agitation at  $100^\circ \text{C}$ . until a uniform mixture is obtained, following which there is added 70 parts of water heated to  $70^\circ \text{C}$ . and a smooth emulsion is obtained. The addition of metallic driers such as the water-soluble salts of a mixture of cobalt, lead and manganese acetates produces a latex varnish which air-dries within four hours when laid down as a film on glass, iron, and aluminum plates. The latex can be pigmented in the usual way to produce high gloss enamels, satin-finish enamels, or semi-gloss and flat-finish paints; or it can be added to other preformed latex paints such as the styrene-butadiene-, acrylic- or vinyl latex paints to improve their adhesion properties.

*Example L*

To 150 parts of dry dioxane containing 40 parts of isoprene, 10 parts of ethyl acrylate and 5 parts of linoleyl vinyl-benzoate, cooled to  $-30^\circ \text{C}$ ., is added 0.3 part of BuLi as a 50% solution in ethyl ether and the mixture maintained at this temperature for 16 hours, following which is neutralized with acetic acid after the mixture is allowed to warm up to room temperature. The dioxane is removed by evaporation at 15 mm. pressure, 120 parts of toluene is added and the resulting polymer solution is filtered.

When metallic driers are added to this solution, and films prepared therefrom, more rapid drying occurs than in a corresponding polymer which contains no linoleyl vinyl-benzoate in its composition.

*Example LI*

To each of 100 parts of oleic acid, linoleic acid and linolenic acid is added 0.1 part of the drier of Example XXIII and glass plates coated with the mixtures. No drying occurs at room temperature in 6 days.

*Example LII*

To each of 100 parts of  $\text{CH}_3\text{COOCH}_2\text{CH}_2\text{OCOC}_{17}\text{H}_{33}$  (prepared from acetic anhydride and hydroxyethyl linole-

ate) and hydroxyethyl linoleate is added 0.1 part of the drier of Example XXIII, and glass plates coated with the mixture as in Example XLII. No drying is observed in 6 days at room temperature.

*Example LIII*

The procedure of Example VII is repeated with the monomers of Examples XV, XVI and XVII and polymerization products are obtained in all cases which air-dry when mixed with the driers of Example XXIII, cast into films and tested as in the procedures of Example LI and LII.

*Example LIV*

In an inert atmosphere, a mixture of 75 parts of styrene and 25 parts of the ether,  $\text{CH}_2=\text{CHC}_6\text{H}_4\text{OC}_{17}\text{H}_{31}$  is added to 200 parts of anhydrous benzene. To this solution is added 0.05 part of BuLi in 1.1 parts of hexane at 25° C. and allowed to react for 24 hours with slow agitation. The mixture is then neutralized with glacial acetic acid and the solution filtered to remove precipitated salts. The copolymer yield is almost quantitative. Titration of the copolymer with bromine for unsaturation shows that the copolymer contains about 24.6% of the ether monomer in the copolymer. Driers are added to the solution and films prepared by the procedure of Example XXIII which air-dry in about 6 hours. To remove volatile matter, the films are dried in an oven at 70-80° C. for 24 hours, then the films tested with 50% aqueous  $\text{H}_2\text{SO}_4$ , conc. HCl, 10% aqueous NaOH, 20% KOH and they remain unaffected, whereas alkyd resin films similarly tested are degraded.

*Example LV*

The procedure of Example XLIV is repeated, using instead of 25 parts of the ether, 25 parts respectively of the hydrocarbons



and  $\text{CH}_2=\text{CHC}_6\text{H}_4\text{CH}_2\text{C}_{17}\text{H}_{31}$  and the corresponding copolymers, respectively, of approximately the same molecular weight are obtained, and they are also very resistant to acids and alkali when their films are air dried.

*Example LVI*

Suitable results are obtained when the procedure of Example VII is repeated a number of times using in place of the sodium equivalent amounts respectively of the following anionic initiators: K, Ca, KH,  $(\text{C}_6\text{H}_5)_3\text{CNa}$ ,  $\text{C}_6\text{H}_5\text{C}(\text{CH}_3)_2\text{K}$ , BuLi,  $\text{C}_6\text{H}_5\text{CH}_2\text{Cs}$ , allyl sodium,  $\text{C}_6\text{H}_5\text{MgBr}$ , BuMgBr, allyl MgBr, and Na naphthyl.

In the above examples, the polymers have repeating unit structures corresponding to the respective monomers used. For example, in Example I, polymers derived from linoleyl vinyl-benzoate having a repeating unit of the formula



polymers derived from the corresponding oleate have a repeating unit of the formula



polymers derived from the corresponding linolenyl ester have a repeating unit of the formula



polymers derived from the corresponding alpha-methyl-

vinyl-benzoates have the repeating units of the following respective formulas



and



In example IX, polymers derived from the vinyl-benzoyl esters of hydroxy-ethyl linoleate and oleate, have the repeating unit formulas respectively:



and



In Example XVIII, polymers derived from the (vinyl-phenoxyl)-ethyl oleate and from the corresponding linoleate have the repeating unit formulas respectively:



and



In Example XXVI, polymers derived from the glyceryl dioleate ester of vinyl-benzoic acid have the repeating unit formula



Polymers derived from the monomer of Example XXVII have repeating units of the formula



While certain features of this invention have been described in detail with respect to various embodiments thereof, it will, of course, be apparent that other modifications can be made within the spirit and scope of this invention, and it is not intended to limit the invention to the exact details shown above except insofar as they are defined in the following claims.

The invention claimed is:

1. A polymer having the plurality of repeating units in the linear chain thereof having a formula



wherein R is selected from the group consisting of hydrogen and methyl;

Ar is a radical having no more than 15 carbon atoms selected from the class consisting of phenylene and the derivatives thereof in which each derivative group is selected from the class consisting of alkyl, aryl, cycloalkyl, alkoxy, aryloxy, cycloalkoxy, carbalkoxy, chlorine, bromine, fluorine,  $-\text{COOCH}_3$ ,  $-\text{COOC}_4\text{H}_9$ ; and amino groups;

Z is a divalent radical of no more than 22 carbon atoms connecting said  $\text{R}_d$  group to said Ar group and contains therein only groups selected from the class consisting of hydrocarbon,  $-\text{C}(\text{O})\text{O}-$ ,  $-\text{O}-$ ,  $-\text{NR}-$  and



groups, in which latter four groups the unoccupied valencies are attached to carbon atoms of groups selected from the class consisting of Ar,  $\text{R}_d$  and a hydrocarbon group of said Z;

$\text{R}_d$  is an unsaturated aliphatic radical containing no less than 16 and no more than 24 carbon atoms and consisting of a terminal  $-\text{CH}_3$  group, at least 1 and no more than 4  $-\text{CH}=\text{CH}-$  groups, and the remainder consisting of  $-\text{CH}_2-$  groups.

2. A polymer of Claim 1, in which said repeating units represent at least 0.1 percent by weight of said polymer.

## 31

3. A polymer of claim 1, in which said repeating units represent at least 0.5 percent by weight of said polymer.

4. A polymer of claim 1, in which said polymer also has a plurality of repeating units therein having the formula



wherein  $\text{Ar}'$  is a monovalent aromatic nucleus.

5. A polymer of claim 1, in which said polymer also has a plurality of repeating units therein having the formula



6. A polymer of claim 1, in which said repeating unit has the formula,



7. A polymer of claim 1, in which said repeating unit has the formula,



8. A polymer of claim 1, in which said repeating unit has the formula,



9. A polymer of claim 1, in which said repeating unit has the formula,



10. A polymer of claim 1, in which said repeating unit has the formula,



11. A polymer of claim 1, in which said repeating unit has the formula,



12. A polymer of claim 1, in which said repeating unit has the formula,



13. A polymer of claim 1, in which said repeating unit has the formula,



14. A polymer of claim 1, in which said repeating unit has the formula,



15. A polymer of claim 1, in which said repeating unit has the formula,



16. A polymer of claim 1, in which said repeating unit has the formula,



17. A polymer of claim 1, in which said repeating unit has the formula,



18. The process of preparing the linear polymer comprising the step of polymerizing a monomer having a

## 32

formula  $\text{CH}_2=\text{C}(\text{R})-\text{Ar}-\text{Z}-\text{R}_d$ , said polymerization being effected in the presence of an anionic initiator at a temperature in the range of  $-80^\circ\text{C}$ . to  $80^\circ\text{C}$ ., in which formulas

5. R is selected from the group consisting of hydrogen and methyl;

Ar is a radical having no more than 15 carbon atoms selected from the class consisting of phenylene and the derivatives thereof in which each derivative group is selected from the class consisting of alkyl, aryl, cycloalkyl, alkoxy, aryloxy, cycloalkoxy, carbalkoxy, chlorine, bromine, fluorine, hydrocarbon carboxylate ester, and amino groups;

Z is a divalent radical of no more than 22 carbon atoms connecting said  $\text{R}_d$  group to said Ar group and contains therein only groups selected from the class consisting of hydrocarbon,  $-\text{C}(\text{O})\text{O}-$ ,  $-\text{O}-$ ,  $-\text{NR}-$  and  $-\text{N}<$  groups, in which latter four groups the unoccupied valencies are attached to carbon atoms of groups selected from the class consisting of Ar,  $\text{R}_d$  and a hydrocarbon group of said Z;

$\text{R}_d$  is an unsaturated aliphatic radical containing no less than 16 and no more than 24 carbon atoms and consisting of a terminal  $-\text{CH}_3$  group, at least 1 and no more than 4  $-\text{CH}=\text{CH}-$  groups, and the remainder consisting of  $-\text{CH}_2-$  groups said anionic initiator being selected from the class consisting of  $\text{NaH}$ ,  $\text{LiH}$ ,  $\text{KH}$ ,  $\text{CsH}$ ,  $\text{LiAlH}_4$ ,  $\text{LiR}^-$ ,  $\text{Nar}^-$ ,  $\text{KR}^-$ ,  $\text{CsR}^-$ ,  $\text{R}^-\text{MgCl}$ ,  $\text{R}^-\text{MgBr}$ ,  $\text{Li}$ ,  $\text{Na}$ ,  $\text{K}$ ,  $\text{Cs}$ ,  $\text{KNH}_2$ ,  $\text{NaNH}_2$ ,  $\text{LiNH}_2$ ,  $\text{Ca}(\text{NH}_2)_2$ ,  $\text{Sr}(\text{NH}_2)_2$  and  $\text{Ba}(\text{NH}_2)_2$ , wherein  $\text{R}^-$  represents a hydrocarbon radical of no more than 12 carbon atoms.

19. The process of claim 12, in which said initiator is sodium.

20. The process of claim 12, in which said initiator is butyl lithium.

21. The process of claim 12, in which said initiator is a combination of sodium and liquid ammonia.

22. A compound having the formula  $\text{CH}_2=\text{C}(\text{R})-\text{Ar}-\text{Z}-\text{R}_d$  wherein R is selected from the group consisting of hydrogen and methyl;

Ar is a radical having no more than 15 carbon atoms selected from the class consisting of arylene radicals and the derivatives thereof in which each derivative group is selected from the class consisting of alkyl, aryl, cycloalkyl, alkoxy, aryloxy, cycloalkoxy, carbalkoxy, chlorine, bromine, fluorine, hydrocarbon carboxylate ester and amino groups;

Z is a divalent radical of no more than 22 carbon atoms connecting said  $\text{R}_d$  group to said Ar group and contains therein only groups selected from the class consisting of hydrocarbon,  $-\text{C}(\text{O})\text{O}-$ ,  $-\text{O}-$ ,  $-\text{NR}-$  and  $-\text{N}<$  groups, in which latter four groups the unoccupied valencies are attached to carbon atoms of groups selected from the class consisting of Ar,  $\text{R}_d$  and a hydrocarbon group of said Z.

$\text{R}_d$  is an unsaturated aliphatic radical containing no less than 16 and no more than 24 carbon atoms and consisting of a terminal  $\text{CH}_3$  group, at least 1 and no more than 4  $-\text{CH}=\text{CH}-$  groups, and the remainder consisting of  $-\text{CH}_2-$  groups.

23. A compound having the formula  $\text{CH}_2=\text{CH}-\text{C}_6\text{H}_4\text{COOC}_{18}\text{H}_{35}$

24. A compound having the formula  $\text{CH}_2=\text{CH}-\text{C}_6\text{H}_4\text{COOC}_{18}\text{H}_{31}$

25. A compound having the formula  $\text{CH}_2=\text{C}(\text{CH}_3)-\text{C}_6\text{H}_4\text{COOC}_{18}\text{H}_{33}$

26. A compound having the formula  $\text{CH}_2=\text{C}(\text{CH}_3)\text{C}_6\text{H}_4\text{COOC}_{18}\text{H}_{35}$

27. A compound having the formula  $\text{CH}_2=\text{C}(\text{CH}_3)\text{C}_6\text{H}_4\text{COOC}_{18}\text{H}_{31}$

28. A compound having the formula  $\text{CH}_2=\text{CHC}_6\text{H}_4\text{COOCH}_2\text{CH}_2\text{OOC}_{17}\text{H}_{31}$

**33**

29. A compound having the formula  
 $\text{CH}_2=\text{CHC}_6\text{H}_4\text{COOCH}_2\text{CH}_2\text{OOCC}_{17}\text{H}_{29}$
30. A compound having the formula  
 $\text{CH}_2=\text{CHC}_6\text{H}_4\text{OCH}_2\text{CH}_2\text{OOCC}_{17}\text{H}_{33}$
31. A compound having the formula  
 $\text{CH}_2=\text{CHC}_6\text{H}_4\text{OCH}_2\text{CH}_2\text{OOCC}_{17}\text{H}_{29}$
32. A compound having the formula  
 $\text{CH}_2=\text{CHC}_6\text{H}_4\text{COOC}_3\text{H}_5(\text{OOC}_{17}\text{H}_{33})_2$

**34**

33. A compound having the formula  
 $\text{CH}_2=\text{CHC}_6\text{H}_4\text{N}(\text{CH}_2\text{COOC}_{18}\text{H}_{33})_2$

No references cited.

5

MURRAY TILLMAN, *Primary Examiner.*  
JAMES E. SEIDLECK, *Examiner.*